

# UNITED STATES PATENT OFFICE.

BENJAMIN B. CROMBIE, OF PORT CHESTER, NEW YORK.

## PROCESS OF PLATINUMIZING METAL SURFACES.

1,274,995.

Specification of Letters Patent.

Patented Aug. 6, 1918.

No Drawing.

Application filed March 29, 1918. Serial No. 225,461.

To all whom it may concern:

Be it known that I, BENJAMIN B. CROMBIE, a citizen of the Dominion of Canada, residing at Port Chester, in the county of 5 Westchester and State of New York, have invented new and useful Improvements in Processes of Platinizing Metal Surfaces, of which the following is a specification.

This invention relates to improvements in 10 means and processes used in depositing a permanent coating of platinum upon the surface of another metal.

The principal object of this invention is 15 to provide a process for plating metals with platinum by the use of chemical and mechanical means only.

A further object is to provide a platinizing means applicable broadly to any metal, which is easily and quickly applied 20 and of the utmost durability, the coating becoming a component part of the metal surface covered by it, indivisible and inseparable, irrespective of its thickness, which depends upon the quantity of composition 25 used.

A still further object is to provide a platinizing compound capable of being used 30 in connection with metals which are difficult to plate by the ordinary electrical deposition of metals, as aluminum, and further, can be applied within the interior of cylindrical and concave metallic articles, that are impossible to plate by usual electrical processes.

These objects are attained by the novel 35 means, processes and principles hereinafter fully described, explained and set forth in the accompanying claims.

The surface of the metallic article to be 40 coated should be clear of oxidization, scale, grease or the like, in fact, both mechanically and chemically clean.

The plating composition consists of a normal platinum chlorid solution ( $PtCl_4$ ) ten 45 parts and a normal ammonium chlorid solution ( $NH_4Cl$ ) eighteen parts forming ammonio platino chlorid, ( $NH_4$ ) ( $2PtCl_6$ ) which is precipitated as a yellow powder.

To one part by weight of the ammonio 50 platino chlorid, add eight parts by weight, of potassium bi-tartrate ( $KHC_4H_4O_6$ ), and three parts by weight of distilled water.

This composition is applied to the polished surface of the metal article to be

plated by a chamois leather dipped in the 55 paste and rubbed vigorously upon the metal surface, the operation being continued or repeated until a desired thickness has been secured.

Obviously the interiors of cylindrical or 60 concave articles in which it is possible to apply the ammonio platino chlorid paste can be effectually covered, as well as the exteriors, as the operation of application is purely mechanical, while adhesion and durability are attained by the chemical affinity 65 action of the paste upon the metal to which it is applied.

The foregoing process renders it possible 70 to coat or plate articles made of base metal, which after being treated, possess substantially all the advantages, appearances and characteristics, of solid platinum, as for instance articles of jewelry, dental goods and laboratory appliances, etc.

If it is desired to produce a highly polished surface, the metallic article, with its 75 first coating of platinum, is placed in a mixture of twelve parts of platinum chlorid, four parts ammonio platino chlorid, and eighty-four parts water, pure platinum foil 80 being used as an anode and the article to be coated as the cathode, and a mild electrical current passed through the solution.

Having thus described my invention and 85 set forth the manner of its use, what I claim as new and desire to secure by Letters Patent, is:—

1. The herein described process of depositing platinum upon metallic surfaces, consisting of the mechanical application of a 90 paste comprised of ammonio platino chlorid one part, potassium bi-tartrate eight parts and distilled water three parts, all substantially as set forth.

2. The herein described process of platinizing metals, consisting of first mechanically and chemically cleansing the metal to be plated, and applying a paste 95 comprised of ammonio platino chlorid one part, potassium bi-tartrate eight parts, and distilled water three parts, by means of a friction pad and continuing until a desired depth of deposition has been attained.

3. The herein described process of platinizing metallic surfaces consisting of cleansing the surface to be plated, rubbing the surface with a paste comprised of am-

monio platino chlorid one part, potassium bi-tartrate eight parts, and distilled water three parts, until the surface is coated and then subjecting the plated article as a 5 cathode in a mixture of twelve parts platinum chlorid, four parts ammonio platino chlorid, and eighty-four parts water, using

an anode of pure platinum foil and passing electric current from the anode to the cathode.

In testimony whereof, I have signed my name to this specification.

BENJAMIN B. CROMBIE.